

May 5, 1953

E. E. PERSHALL

2,637,691

WOOD PRESERVATION

Filed July 16, 1951



*E. E. Pershall,  
Inventor  
Koenig and Pope,  
Attorneys*

## UNITED STATES PATENT OFFICE

2,637,691

## WOOD PRESERVATION

Estes E. Pershall, Hazelwood, Mo., assignor to  
 T. J. Moss Tie Company, St. Louis, Mo., a corporation of Missouri

Application July 16, 1951, Serial No. 236,994

9 Claims. (Cl. 252—8.1)

1

This invention relates to wood preservation and more particularly to treated wood materials, treating solutions therefor, and the manufacture of such materials and solutions.

This application is a continuation-in-part of copending applications, Serial Nos. 38,164 and 38,165, both filed July 10, 1948.

Briefly, this invention is directed to wood through which is distributed an ammoniated basic zinc chloride having an average ratio of zinc to chlorine greater than that in zinc chloride, and to ammoniated basic zinc chloride treating solutions for rendering wood fire-resistant. Methods of rendering wood fire-resistant with these treating solutions are also within the scope of the present invention.

Among the several objects of this invention are the provision of treated wood materials which are resistant to fire, fungi and insects; the provision of materials of the class described which are not only initially highly resistant to fire but which retain a substantial portion of such fire resistance after extensive exposure to leaching and weathering action; the provision of treated wood materials which are free from objectionable odor, paintable and safe to handle; the provision of treating solutions for wood materials which are safe to handle and are not detrimental to the mechanical properties of the wood or the natural appearance thereof; the provision of treating solutions of the class described which are convenient to handle, economical to prepare and convenient to introduce into the material to be treated; and the provision of methods of rendering wood fire-resistant with such treating solutions which are convenient, efficient and economical. Other features will be in part apparent and in part pointed out hereinafter.

The invention accordingly comprises the products and methods hereinafter described, the scope of the invention being indicated in the following claims.

In the accompanying drawing the single figure graphically illustrates the relationship between the fire resistance both before and after leaching of the treated woods of this invention and the composition ratio of the ammoniated basic zinc chloride treating solutions at various values of retention.

Wood is a highly useful material but it possesses two inherent disadvantages, inflammability and susceptibility to deterioration by fungi and insects. Many different methods have been proposed and used to remedy one or both of these faults, but none has been completely satisfac-

2

tory in providing a treated wood product which will withstand leaching to any substantial extent. Thus, the use of these prior-art treatments is limited to conditions where the treated wood is not frequently subjected to heavy rainfall, condensation or other contact with water in one form or another.

In accordance with the present invention, however, it has been found that wood products can be made which are fire-resistant (initially as well as after leaching), insect and fungi-resistant, free from objectionable odor, paintable, and safe to handle. These novel wood products contain an ammoniated basic zinc chloride distributed therethrough and are formed by impregnating wood with a treating solution of the present invention. By ammoniated basic zinc chloride is meant a composition which may include a number of compounds and not a single compound with a definite zinc to chlorine ratio.

The treating solutions described and claimed herein are not detrimental to the mechanical properties and natural appearance of the wood. These treating solutions are ammoniacal solutions of a basic zinc chloride, i. e. complexes of zinc chloride and zinc oxide with ammonia. By basic zinc chloride, I mean a zinc chloride which has an average ratio of zinc to chlorine greater than that in zinc chloride. That is, there must be more than one atom of zinc present for each two atoms of chlorine in these ammoniated basic zinc chloride treating solutions, and the excess of zinc must be combined with oxygen or hydroxyl. Preferably, these ammoniated basic zinc chlorides have a basicity represented by a composition on the dry basis of greater than approximately  $.2\text{ZnO:1ZnCl}_2:2\text{NH}_3$ . By basicity is meant the amount of zinc oxide or hydroxide combined with zinc chloride. Even more preferable are ammoniated basic zinc chlorides having a composition on the dry basis between approximately  $.2\text{ZnO:1ZnCl}_2:2\text{NH}_3$  and

$4\text{ZnO:1ZnCl}_2:2\text{NH}_3$

and more specifically about

$2\text{ZnO:1ZnCl}_2:2\text{NH}_3$

The concentration of the ammoniated basic zinc chloride in the ammonium hydroxide may be varied considerably and is determined by factors such as the solubility of the particular basic zinc chloride in ammonium hydroxide and the concentration of the ammonium hydroxide solvent. Generally, the higher the basicity of the particular basic zinc chloride utilized, the lower

is its solubility in ammonium hydroxide. It is preferred that the concentration of these basic zinc chlorides in ammonium hydroxide (on the dry basis by weight) be about 16% to 18% and that the concentration of the ammonium hydroxide be in the order of about 20% ammonia. Lower and higher concentrations of the ammoniated basic zinc chloride and of the ammonium hydroxide are of course within the scope of the invention.

Wood impregnated with the treating solutions of this invention is fire-resistant both before and after leaching. Fire-resistant wood is defined herein as wood which will lose not more than 55% of its weight during a standard fire-tube test (as determined by the method prescribed and approved by the United States Department of Agriculture Forest Service, Forest Products Laboratories in Madison, Wisconsin, in the 1931 article "The 'Fire-proofing' of Wood" by T. R. Truax, Senior Wood Technologist, published in the 1931 Proceedings of the Fire Protection Association). Treated wood which loses not more than 30% of its weight in this test is considered highly fire-resistant.

The degree of fire resistance of the treated wood of this invention is dependent upon such factors as the amount and concentration of treating solution retained (on a dry basis) in the wood and to some extent on the basicity of the ammoniated basic zinc chloride in the treating solution. Generally, the greater the amount and/or the higher the concentration of treating solution, the greater will be the retention and the greater the fire resistance of the treated wood.

The concentration of the ammoniated basic zinc chloride in the treating solution will determine whether single or multiple impregnations are necessary to distribute the desired amount of ammoniated basic zinc chlorides through the wood. For example, in relatively soft woods, such as white pine, about 3.5 pounds of ammoniated basic zinc chloride (on the dry basis) will be retained per cubic foot of the untreated wood after a single impregnation if the concentration of the ammoniated basic zinc chloride in the treating solution is approximately 10% by weight. If a treating solution having a lower concentration of ammoniated basic zinc chloride, such as 6% to 8%, is used it may be necessary to impregnate the wood several times to obtain a retention in the order of 3.5 pounds per cubic foot.

The fire resistance of the treated wood of this invention prior to weathering or leaching does not appear to be appreciably affected by the basicity of the particular ammoniated basic zinc chloride with which it is impregnated, but only by the amount retained. This relationship of initial fire-tube loss to basicity is illustrated in the drawing, curve A-1 representing a retention of three pounds of the ammoniated basic zinc chloride treating solution on the dry basis per cubic foot of the wood treated. Curves B-1 and C-1 are similar to A-1 but represent constant retentions of four and five pounds per cubic foot, respectively.

However, the basicity of the particular ammoniated basic zinc chloride employed appears to have an effect on the degree of fire resistance of the treated wood after leaching. It has been found that the fire-tube loss (at a constant value of retention) after leaching will vary with the basicity of the ammoniated basic zinc chlorides and be an optimum (i. e. minimum) at a value

of about  $2\text{ZnO}:1\text{ZnCl}_2:2\text{NH}_3$ . This is illustrated by curves A-2, B-2 and C-2 representing the relationship between fire-tube loss after leaching for 15 days and basicity, at three, four and five pounds per cubic foot retention, respectively. The optimum may vary somewhat depending upon the evaporation conditions.

Thus, wood containing about 5.5 pounds or more of these novel ammoniated basic zinc chlorides (on the dry basis) per cubic foot will, in general, have a fire-tube loss of about 20% or less prior to leaching and less than 55% subsequent to leaching. If even higher degrees of fire resistance are desired greater retentions such as 14 to 16 pounds per cubic foot may be used without detriment to the properties of the wood thus treated. On the other hand, wood impregnated with lesser amounts of these ammoniated basic zinc chlorides is also fire-resistant, and at retentions such as about 3.5 pounds per cubic foot, the fire-tube loss prior to leaching will not usually run more than about 30%.

These novel treating solutions are made in accordance with this invention by forming an ammoniacal solution of basic zinc chloride which has an average ratio of zinc to chlorine greater than that in zinc chloride. The basic zinc chloride may be formed by intermixing zinc oxide, zinc chloride and water to form a basic zinc chloride and thereafter dissolving it in aqueous ammonia. The amount of water intermixed with zinc chloride and zinc oxide may be varied considerably without detriment to the basic zinc chloride formed. For example, if the amount of water used is about 10% of the weight of the final zinc oxide-zinc chloride-water mixture a cement-like form of basic zinc chloride is formed, whereas if a higher percentage of water such as about 25% is used, then a mud-like form of basic zinc chloride results. If even greater amounts of water are employed in the water-zinc oxide-zinc chloride mix, such as for example 50%, then a slurry-like form of basic zinc chloride results. Alternately, zinc chloride solution or a zinc oxide slurry may be added to dry zinc oxide or dry zinc chloride, respectively, to form the basic zinc chlorides. Similarly, zinc oxide in a finely ground state may be added to a hot aqueous zinc chloride solution which is then cooled to form a basic zinc chloride precipitate. This precipitate is subsequently dissolved in ammonium hydroxide. Also, zinc chloride and zinc oxide may be intermixed with ammonium hydroxide to form an ammoniated basic zinc chloride treating solution. The basicity of the resulting ammoniated basic zinc chlorides may be varied by varying the ratio of zinc oxide to zinc chloride reactants.

As a further modification of the method of making these treating solutions, zinc chloride is mixed with ammonium hydroxide (the latter in excess over a 1:2 mole ratio of zinc chloride to ammonium hydroxide) and a fixed alkali or base (i. e. any non-volatile alkaline hydroxide such as potassium, sodium and barium hydroxides) is added to form an ammoniated basic zinc chloride treating solution. The basicity or ratio of zinc oxide to zinc chloride, is dependent upon the amount of base added.

The following examples illustrate the invention.

#### Example 1

An aqueous solution of approximately 80% zinc chloride by weight was heated and zinc oxide was added in a proportion of approximately 5%

of the weight of the zinc chloride present in the solution. The zinc oxide-zinc chloride-water solution was then cooled and a basic zinc chloride having a composition of approximately  $1\text{ZnO}:1\text{ZnCl}_2:\text{XH}_2\text{O}$  separated from the solution as a precipitate. This precipitated salt was filtered from the solution and washed with a small amount of water, and then dissolved in aqueous ammonia of approximately 25% concentration, by weight. A treating solution was made by diluting the above ammoniated basic zinc chloride solution with water until the content thereof was approximately 16-18% of ammoniated salt in 12-15% aqueous ammonia solution. The composition of this soluble ammoniated basic zinc chloride salt on a dry basis (when dried at approximately 75° C.) was approximately



*Example 2*

15,000 grams of zinc chloride was dissolved in 10,000 milliliters of water to make a 60% solution. This solution was heated to boiling and 1,500 grams of zinc oxide was slowly added. Heating was continued until the zinc oxide was in solution. The solution was allowed to cool to room temperature. The precipitate, a basic zinc chloride, was filtered off, washed and dissolved in 28% aqueous ammonia. A treating composition was made by diluting the above ammoniated basic zinc chloride solution with water until the content thereof was approximately 16-18% of ammoniated salt in 12-15% aqueous ammonia solution. The composition of the ammoniated basic zinc chloride salt on the dry basis (when dried at approximately 75° C.) was approximately  $.6\text{ZnO}:1\text{ZnCl}_2:2\text{NH}_3$ .

*Example 3*

A 50% aqueous solution of zinc chloride by weight was heated and zinc oxide was added to this solution in a proportion of approximately 5% of the weight of the zinc chloride present in the solution. This solution was then allowed to cool and a basic zinc chloride having a composition of approximately  $2.5\text{ZnO}:1\text{ZnCl}_2:\text{XH}_2\text{O}$  separated from the solution as a precipitate. This basic zinc chloride salt was then dissolved in aqueous ammonia solution to give an ammoniated basic zinc chloride having a composition on a dry basis (when dried at approximately 75° C.) of approximately  $1.6\text{ZnO}:1\text{ZnCl}_2:2\text{NH}_3$ . A treating composition was made by diluting the above ammoniated basic zinc chloride solution with water until the content thereof was approximately 16-18% of ammoniated salt in 12-15% aqueous ammonia solution.

*Example 4*

20 pounds of dry zinc chloride and 6.56 pounds of dry zinc oxide were intimately mixed until a smooth powder was obtained. This gave a homogeneous mixture having a molecular ratio of  $.55\text{ZnO}:1\text{ZnCl}_2$ . Water was added in approximately 1 pound increments until a total of 9 pounds of water had been added. The resulting mixture had the consistency of a thick mud. All large lumps formed during the addition of water were broken and dispersed so that a homogeneous mixture was obtained. The above mixture of basic zinc chloride was aged six days and then intimately mixed with 55 pounds of aqueous ammonia containing 25% ammonia by weight. The solution was then filtered to remove any undissolved solids, such as undissolved zinc oxide. The

filtrate was diluted to a strength of 16-18% solids in 12-15% aqueous ammonia. The composition of this ammoniated basic zinc chloride solution on a dry basis (when dried at approximately 75° C.) was approximately  $.3\text{ZnO}:1\text{ZnCl}_2:2\text{NH}_3$ .

*Example 5*

8 pounds of zinc chloride and 3 pounds of water were intimately mixed until a solution was obtained. 7.16 pounds of zinc oxide was added and the resulting cement-like mixture was mixed until a homogeneous dispersion was obtained. This gives a homogeneous mixture having a molecular ratio of  $1.5\text{ZnO}:1\text{ZnCl}_2$ . The above mixture of basic zinc chloride was intimately mixed with 40 pounds of 25% (by weight) aqueous ammonia, and the resulting solution was filtered to remove any undissolved solids, such as undissolved zinc oxide. The filtrate was diluted to a strength of 16-18% solids in 12-15% aqueous ammonia. The composition of this ammoniated basic zinc chloride solution on a dry basis (when dried at approximately 75° C.) was approximately  $.95\text{ZnO}:1\text{ZnCl}_2:2\text{NH}_3$ .

*Example 6*

8.95 pounds of zinc oxide and 15 pounds of water were intimately mixed until a slurry was obtained. 20 pounds of zinc chloride was added and the resulting cement-like mixture was mixed until a homogeneous dispersion was obtained. The molecular ratio of this mixture was approximately  $.75\text{ZnO}:1\text{ZnCl}_2$ . The above mixture of basic zinc chloride was intimately mixed with 70 pounds of 25% (by weight) aqueous ammonia, and the resulting solution was filtered to remove any undissolved solids, such as undissolved zinc oxide. The filtrate was diluted to a strength of 16-18% solids in 12-15% aqueous ammonia. The composition of this ammoniated basic zinc chloride solution on a dry basis (when dried at approximately 75° C.) was approximately



*Example 7*

2385 grams of zinc oxide was placed in a ball mill and a solution of 1000 grams of zinc chloride dissolved in 1500 milliliters of water was sprayed over the zinc oxide while milling for 10 minutes. 40 pounds of commercial concentrated aqueous ammonia (28%) was added and milling was continued for another 10 minutes to dissolve the reaction product. The solution was filtered to remove any undissolved solids.

55 This solution contained 12.89% by weight of an ammoniated basic zinc chloride having a composition on the dry basis (when dried at approximately 75° C.) of  $2.35\text{ZnO}:1\text{ZnCl}_2:2\text{NH}_3$  dissolved in ammonium hydroxide.

*Example 8*

A solution of 300 grams of zinc chloride dissolved in 700 milliliters of water was added to 700 milliliters of 28% aqueous ammonia. A solution of 132 grams of sodium hydroxide dissolved in 150 milliliters of water and 150 milliliters of 28% aqueous ammonia was added to the ammoniacal zinc chloride solution to produce a treating solution of 12.1% by weight of an ammoniated basic zinc chloride having a composition on the dry basis (when dried at approximately 75° C.) of  $1.5\text{ZnO}:1\text{ZnCl}_2:2\text{NH}_3$  dissolved in ammonium hydroxide.

*Example 9*

An aqueous solution of zinc chloride and an

aqueous slurry of zinc oxide were mixed in a tank with agitation to form a mixture containing 12 pounds of zinc oxide, 40 pounds of zinc chloride and 60 pounds of water. The tank was sealed and this mixture was agitated for 5 days intermittently during which time 41.4 pounds of anhydrous ammonia gas was introduced intermittently to maintain an average pressure of about 50 pounds per square inch and an average temperature of 85° F. The resulting solution was 39.29% by weight of an ammoniated basic zinc chloride having a composition on a dry basis (when dried at approximately 75° C.) of



dissolved in ammonium hydroxide.

*Example 10*

1895 grams of zinc oxide were placed in a ball mill and a solution of 1275 grams zinc chloride dissolved in 1275 milliliters of water was sprayed over the zinc oxide while milling for 10 minutes. 35 pounds of commercial concentrated aqueous ammonia were added and milling was continued for another 10 minutes. The solution was filtered to remove any undissolved solids.

This solution contained 14.2% by weight of an ammoniated basic zinc chloride having a composition on the dry basis (when dried at approximate 75° C.) of 2.0ZnO:1ZnCl<sub>2</sub>:2NH<sub>3</sub> dissolved in ammonium hydroxide.

*Example 11*

2390 grams of calcium hydroxide was placed in a ball mill and a solution of 4000 grams of zinc chloride dissolved in 4000 milliliters of water was added while milling. A precipitate was formed, washed by decantation and filtered. 7.5 pounds of anhydrous ammonia was added to the wet filter cake (34.2 pounds). The resultant mixture was filtered to remove any undissolved solids.

This solution contained 9.6% by weight of an ammoniated basic zinc chloride having a composition on the dry basis (when dried at approximately 75° C.) of 4.0ZnO:1ZnCl<sub>2</sub>:2NH<sub>3</sub> dissolved in ammonium hydroxide.

*Example 12*

A sample wood stick (cut to the standard dimensions described and approved by the United States Department of Agriculture Forest Service, Forest Products Laboratories in Madison, Wisconsin, in the 1931 article "The Fire-proofing of Wood," published in 1931 Proceedings of the Fire Protection Association by T. R. Truax, Senior Wood Technologist) was impregnated with the ammoniated basic zinc chloride solution of Example 1 by any conventional treating apparatus until the retention was approximately 7.7 pounds of ammoniated basic zinc chloride salt per cubic foot of the wood sample. The wood thus treated was highly fire-resistant, paintable, free from objectionable odor, possessed of desirable mechanical and chemical properties and retained a high degree of fire resistance after exposure to leaching. Such treated wood sample had initially a fire-tube loss (as determined by the method described and approved by the Forest Products Laboratories in the 1931 article cited above) of approximately 17%, and after leaching the sample totally submerged in briskly running water (e. g., water is completely changed at least every 2 hours) for 15 days, approximately 20%. After 30 days leaching the fire-tube loss was only approximately 22%. 75

*Example 13*

A sample wood stick was impregnated with the ammoniated basic zinc chloride solution of Example 2 by any conventional treating apparatus until the retention was approximately 5 pounds of the ammoniated basic zinc chloride salt per cubic foot of wood. The wood thus treated was highly fire-resistant, paintable, free from objectionable odor, possessed of desirable mechanical and chemical properties and retained a high degree of fire resistance after exposure to leaching. Such treated wood had initially a fire-tube loss of not more than 20% and after leaching totally submerged in briskly running water for 15 days, not more than 30%.

*Example 14*

A sample wood stick was impregnated with the ammoniated basic zinc chloride composition of Example 3 until the retention was approximately 7.7 pounds of ammoniated salt per cubic foot of the wood sample. The wood thus treated was highly fire-resistant, paintable, free from objectionable odor, possessed of desirable mechanical and chemical properties and retained a high degree of fire resistance after exposure to leaching. Such treated wood had initially a fire-tube loss of not more than 20% and after leaching totally submerged in briskly running water for 15 days, not more than 30%.

*Example 15*

A sample wood stick was impregnated with the ammoniated basic zinc chloride solution of Example 4 by any conventional treating apparatus until the retention was approximately 6.74 pounds of ammoniated basic zinc chloride salt per cubic foot of the wood sample. The wood thus treated was highly fire-resistant, paintable, free from objectionable odor, possessed of desirable mechanical and chemical properties and retained a high degree of fire resistance after exposure to leaching. Such treated wood sample had initially a fire-tube loss of approximately 15% (as determined by the method described and approved by the Forest Products Laboratories in the 1931 article cited above), and after leaching the sample totally submerged in briskly running water for 15 days, approximately 25%.

*Example 16*

A sample wood stick was impregnated with the ammoniated basic zinc chloride solution of Example 5 by any conventional treating apparatus until the retention was approximately 5.6 pounds of the ammoniated basic zinc chloride salt per cubic foot of wood. The wood thus treated was highly fire-resistant, paintable, free from objectionable odor, possessed of desirable mechanical and chemical properties and retained a high degree of fire resistance after exposure to leaching. Such treated wood has initially a fire-tube loss of approximately 20% and after leaching in running water for 15 days, approximately 27%. After 30 days leaching the fire-tube loss was only 30%.

*Example 17*

A sample wood stick was impregnated with the ammoniated basic zinc chloride composition of Example 6 until the retention was approximately 5.3 pounds of ammoniated salt per cubic foot of wood sample. The wood thus treated was highly fire-resistant, paintable, free from objectionable odor, possessed of desirable mechanical and chemical properties and retained a high degree of fire resistance after exposure to leaching. Such

treated wood had initially a fire-tube loss of approximately 20% and after leaching in running water for 15 days approximately 29%.

*Example 18*

The procedure of Example 12 was followed using the treating solution of Example 7. The characteristics of the treated wood stick were similar to those described in Example 12 except that at a retention of 5.5 pounds per cubic foot the initial fire-tube loss was 17% and after 15 days of leaching it was 22%.

*Example 19*

The procedure of Example 12 was followed using the treating solution of Example 8. The characteristics of the treated wood stick were similar to those described in Example 12 except that at a retention of 5 pounds per cubic foot the initial fire-tube loss was 20% and after 15 days of leaching it was 32%.

*Example 20*

The procedure of Example 12 was followed using the treating solution of Example 9. The characteristics of the treated wood stick were similar to those described in Example 12 except that at a retention of 4.3 pounds per cubic foot the initial fire-tube loss was 19% and after 15 days of leaching it was 48%.

*Example 21*

The procedure of Example 12 was followed using the treating solution of Example 10. The characteristics of the treated wood stick were similar to those described in Example 12 except that at a retention of 5.2 pounds per cubic foot the initial fire-tube loss was 18% and after 15 days of leaching it was 25%.

*Example 22*

The procedure of Example 12 was followed using the treating solution of Example 11. The characteristics of the treated wood stick were similar to those described in Example 12 except that at a retention of 8 pounds per cubic foot the initial fire-tube loss was 18% and after 15 days of leaching it was 23%.

Any customary method of impregnation may be employed for treating wood with the treating solutions of the present invention.

It is to be understood that in addition to the ratio of  $ZnO$  to  $ZnCl_2$  in the above compositions being variable as stated, variations in the conditions of evaporation of the treating solution to a dry basis will vary the ratio of  $NH_3$  to  $ZnCl_2$ .

It is also to be understood that ammoniated basic zinc chlorides having higher ratios than  $4ZnO:1ZnCl_2:2NH_3$ , such as  $7ZnO:1ZnCl_2:2NH_3$  and  $10ZnO:1ZnCl_2:2NH_3$ , have been made and used successfully in carrying out the present invention.

In view of the above, it will be seen that the several objects of the invention are achieved and other advantageous results attained.

As many changes could be made in the above methods and products without departing from the scope of the invention, it is intended that all matter contained in the above description shall be interpreted as illustrative and not in a limiting sense.

I claim:

1. A treating solution for rendering wood fire-

resistant before and after leaching with water comprising an ammoniacal solution of an ammoniated basic zinc chloride having a composition on the dry basis between approximately

5  $.2ZnO:1ZnCl_2:2NH_3$

and  $4ZnO:1ZnCl_2:2NH_3$ .

10 2. A treating solution for rendering wood fire-resistant before and after leaching with water comprising an ammoniacal solution of an ammoniated basic zinc chloride having a composition on the dry basis of approximately

$2ZnO:1ZnCl_2:2NH_3$

15 3. A treating solution for rendering wood fire-resistant before and after leaching with water comprising an ammoniacal solution of an ammoniated basic zinc chloride having a composition on the dry basis between approximately

20  $.2ZnO:1ZnCl_2:2NH_3$  and  $4ZnO:1ZnCl_2:2NH_3$ , the concentration of said ammoniated basic zinc chloride in said solution being at least approximately 10% by weight.

25 4. A treating solution for rendering wood fire-resistant before and after leaching with water comprising an ammoniacal solution of an ammoniated basic zinc chloride having a composition on the dry basis between approximately

30  $.2ZnO:1ZnCl_2:2NH_3$ , and  $4ZnO:1ZnCl_2:2NH_3$ , the concentration of said ammoniated basic zinc chloride in said solution being at least approximately 16% to 18%.

35 5. A treating solution for rendering wood fire-resistant before and after leaching with water comprising an ammoniacal solution of an ammoniated basic zinc chloride having a composition on the dry basis of approximately

$2ZnO:1ZnCl_2:2NH_3$

40 40 the concentration of said ammoniated basic zinc chloride in said solution being approximately 16% to 18% in approximately 20% ammonium hydroxide.

45 45 6. Wood which is fire-resistant before and after leaching with water comprising the product resulting from the impregnation and drying of wood with an ammoniacal solution of an ammoniated basic zinc chloride having a composition on the dry basis between approximately

$.2ZnO:1ZnCl_2:2NH_3$

and approximately  $4ZnO:1ZnCl_2:2NH_3$ .

50 55 7. Wood which is fire-resistant before and after leaching with water comprising the product resulting from the impregnation and drying of wood with an ammoniacal solution of an ammoniated basic zinc chloride having a composition on the dry basis of approximately

$2ZnO:1ZnCl_2:2NH_3$

60 65 8. Wood which is fire-resistant before and after leaching with water comprising the product resulting from the impregnation and drying of wood with an ammoniacal solution of an ammoniated basic zinc chloride to obtain a retention of at least approximately 3.5 pounds per cubic foot on the dry basis, said ammoniated basic zinc chloride having a composition on the dry basis between approximately  $.2ZnO:1ZnCl_2:2NH_3$  and approximately  $4ZnO:1ZnCl_2:2NH_3$ .

70 70 9. Wood which is fire-resistant before and after leaching with water comprising the product resulting from the impregnation and drying of wood with an ammoniacal solution of an am-

11

moniated basic zinc chloride to obtain a retention of at least approximately 5.5 pounds per cubic foot on the dry basis, said ammoniated basic zinc chloride having a composition on the dry basis of approximately  $2\text{ZnO} \cdot 1\text{ZnCl}_2 \cdot 2\text{NH}_3$ .

ESTES E. PERSHALL.

References Cited in the file of this patent

## UNITED STATES PATENTS

|         |          |              |
|---------|----------|--------------|
| Number  | Name     | Date         |
| 959,505 | Gerlache | May 31, 1910 |

5.

|        |           |
|--------|-----------|
| Number | 1,261,736 |
|        | 1,318,524 |
|        | 1,338,322 |

|              |              |               |
|--------------|--------------|---------------|
| Name         | Ferguson     | Date          |
|              | Apr. 2, 1918 |               |
| Arent et al. |              | Oct. 14, 1919 |
| Munroe       |              | Apr. 27, 1920 |

10.

|          |                                                                                                                            |
|----------|----------------------------------------------------------------------------------------------------------------------------|
| Number   | 10                                                                                                                         |
| Name     | Mellor                                                                                                                     |
| and 549. | "Comprehensive Treatise on Inorganic and Theoretical Chemistry"—Longmans, Green and Co.—London—1929—Vol. 4, pages 545, 546 |

## OTHER REFERENCES

Mellor—"Comprehensive Treatise on Inorganic and Theoretical Chemistry"—Longmans, Green and Co.—London—1929—Vol. 4, pages 545, 546 and 549.

12